

Patented Sept. 22, 1925.

1,554,629

# UNITED STATES PATENT OFFICE.

HARRY B. GOODWIN, OF GRAND JUNCTION, COLORADO, ASSIGNOR TO THE LATIMER-GOODWIN CHEMICAL COMPANY, OF GRAND JUNCTION, COLORADO, A CORPORATION OF COLORADO.

## SPREADER FOR INSECTICIDAL COMPOSITIONS AND THE LIKE.

No Drawing.

Application filed December 6, 1923. Serial No. 679,000.

To all whom it may concern:

Be it known that I, HARRY B. GOODWIN, a citizen of the United States, and a resident of Grand Junction, county of Mesa, 5 and State of Colorado, have invented a new and useful Improvement in Spreaders for Insecticidal Compositions and the like, of which the following is a specification, the principle of the invention being herein explained and the best mode in which I have contemplated applying that principle, so as to distinguish it from other inventions. With the almost universal adoption of dry powdered lead arsenate as a spray material for the control of leaf-eating insects, 15 the manufacture of this material has become practically standardized as regards its chemical composition. With no further improvement to be looked for on the chemical side, attention has been directed toward the improvement of the water-lead arsenate spray mixture so as to make it a more efficient agent. Work in this field has followed 20 two lines of development, the first being an effort to improve the physical properties of the solid lead arsenate, and the second being an effort to improve the liquid or water phase of the system.

Quite early in the manufacture of powdered lead arsenate it was noticed that the fine particles tended to cohere, forming groups or flakes when the material was suspended in water. These flakes are objectionable for two reasons. In the first place, 25 a cluster of particles will not cover as much surface as the individual particles uniformly dispersed through the liquid, and second, the clusters in suspension behave like solid particles of relatively large size in 30 that they settle out of the water rapidly.

As disclosed in U. S. Letters Patent No. 1,322,008, granted to me under date of November 18, 1919, the addition of a colloid, specifically a relatively chemically inert 45 colloid of organic origin, of which tannin is a preferred example, to dry lead arsenate will overcome this tendency to cluster and produce a spray mixture in which the particles are practically as finely divided as 50 at the time of their formation in the precipitating tank. The use of such a deflocculator, in other words, gives a spray mixture in which the lead arsenate particles are evenly dispersed and they remain in sus-

pension for a much longer time. Such deflocculator requires to be used in very small amounts only, as little as  $\frac{1}{2}$  lb. of tannin to 100 lbs. of lead arsenate producing satisfactory results. Other deflocculating agents that may be used with satisfactory results 60 are gum arabic, glue or gelatin and alkali metal salts of casein, specifically sodium caseinate.

The efforts to make the water a more effective agent have been along the line of 65 reducing the surface tension of the liquid. The fruit and leaves of plants acquire a wax-like covering as the season advances and when a water-lead arsenate spray is applied in the usual manner, the fog of 70 spray tends to draw together in drops instead of spreading out in a thin layer.

Materials added for the purpose of thus increasing the wetting and covering power of the spray solution have been appropriately termed "spreaders" by Prof. A. L. Lovett who has investigated a number of substances in regard to their desirability for this purpose, as reported in Oregon Agricultural College Experiment Station Bulletin 169. The materials named in the foregoing bulletin as showing value as spreaders in the poison spray solution given in order of their merit, based on compatibility, 75 efficiency, availability, cost and ease of preparation, are:—caseinate, glue, gelatin, soap bark and oil emulsions. Since the publication of Dr. Lovett's work (1920), there has grown up a very considerable business in the manufacture and sale of lime casein 80 mixtures to be added to spray tanks. The quantities in which this material is sold is evidence that fruit growers believe they are obtaining better results through its use.

In order to be wholly satisfactory, a 85 spreader should possess the following properties, viz, (1) it must not affect the spray material, fruit or foliage injuriously; (2) it should be effective in small quantities; (3) it should be salable in dry form; (4) it should be quickly and completely soluble in cold water; and (5) it should be a chemical compound. If the above be taken as the properties to be possessed by a perfect 90 spreader, then all of the materials so far suggested for this use have one or more 95 counts against them. As a result, however, of prolonged and careful investigation, I 100

have found that certain substances belonging to the class of so-called gum-resins appear to be best suited for this purpose. As examples of such gum-resins, olibanum, 5 myrrh, mastic and gamboge may be mentioned, but the last named appears to be satisfactory to a most unusual degree. The foregoing materials and particularly gamboge will now be set forth with some particularity, it being understood, however, both as to the ingredients employed in my improved spreading material and as to the method of making and using same, that changes may be made therein without departing from the spirit of the invention. 10 15

Gamboge, also written gambooge, is the inspissated juice of various species of the guttiferous genus *Garcinia*, the gamboge of commerce being mainly derived from *G. Hanburyi* which is a native of Siam, Cambodia and Cochin, China. It is a gum-resin product, the only uses of which heretofore have been in medicine where it acts as a drastic purgative and as a pigment in water- 20 25 30 35 40 45 50 55 60 65 color painting for the production of transparent yellows verging on brown in deep masses. For use as a spreader with water mixtures of calcium arsenate and other insecticidal compositions that have sufficient alkalinity to dissolve gamboge, the commercial product may be directly employed, but preferably I convert the same into the form of an alkali metal salt, specifically sodium gamboge. As an example of such conversion, I add to 100 lbs. of gamboge 12½ lbs. of sodium hydrate, 3.2 ounces of potassium dichromate, and enough water to make a stiff paste. By means of suitable apparatus, which need not be described, the materials are kneaded or rubbed into a uniform paste without lumps, no heat being required. Such paste is then dried in warm air at about 130 degrees F., but any standard method for drying materials of similar nature may be employed. The resultant dry cake is then pulverized in a suitable mill, the product being a finely divided powder varying in color from yellow to light brown.

Instead of adding only enough water to form a paste, a greater quantity of water may be used so that the ingredients are all in solution and this solution can then be boiled until the excess water is removed and a paste formed, the final water in the paste then being removed by drying at a lower temperature as before. Other oxidizing agents than potassium dichromate may be used, such for example as sodium dichromate, hydrogen peroxide, sodium peroxide, sodium nitrate, sodium perchlorate, potassium permanganate, the choice being determined by the market price, permanency and ease of handling. The dichromate is preferable because it is a dry salt that does not lose its oxidizing power under normal conditions;

furthermore it is not deliquescent and has no fire or explosion risk.

As a basis for determining the relative efficiency of the foregoing new composition of matter and other substances as spreaders, 70 I have employed the interfacial tension apparatus developed by A. W. Fahrenwald as reported in the Journal of the Optical Society of America and Review of Scientific Instruments, vol. 6, No. 7, Sept. 1922. A 75 paraffin oil having a specific gravity of 0.885 was used as a surface layer in all of the experiments and in preparing the substances for examination, the following procedure was followed, viz, 0.3 grams of such substance were dissolved in distilled water and diluted to 250 cc. in a graduated flask, this representing 2 lbs. of spreader in 200 gallons of water or 50 per cent of the arsenate of lead power on the assumption that 4 lbs. 80 is the usual amount of the latter added to a 200 gallon tank. After mixing, half of this spreader solution was used to obtain the result in an appropriately designated column of the subjoined tabulated statement. The other half was diluted to 250 cc. in the same flask, thus giving the equivalent of 1 lb. of spreader to 200 gallons or 25 per cent of lead arsenate when used in the usual spray strength. The results in this case, as also 85 in the case where the spreader is employed in an amount equivalent to 5 per cent and in an amount equivalent to ½ of 1 per cent of the lead arsenate, respectively, are likewise shown in the table which follows. 90 95 100

For the purpose of comparison, corresponding tests with other substances heretofore used or suggested for use as spreaders are tabulated along with the results obtained with sodium gamboge, it being noted that the interfacial tension of the oil and distilled water employed in these tests at room temperature was 31 dynes. 105

#### *I. Interfacial tension of various spreaders (in dynes per cm.).*

| Amount of spreader in 200 gallons water | 0.02 lb. | 0.2 lb. | 1 lb. | 2 lbs. | 110 |
|-----------------------------------------|----------|---------|-------|--------|-----|
| Tannin                                  | 30       | 29      | 28    | 23     |     |
| Sodium caseinate (dry)                  | 31       | 28      | 23    | 21     |     |
| Glue (Armour's 631543)                  | 31       | 28      | 24    | 21     |     |
| Gum arabic                              | 31       | 31      | 31    | 31     |     |
| sodium gamboge                          | 13       | 11      | 8     | 7      | 115 |

From the foregoing, the marked superiority of sodium gamboge, even when employed in an amount equivalent to only 5 per cent of the dry lead arsenate, will be immediately apparent. 120

While sodium gamboge is thus shown to be a superior agent for the reduction of the surface tension of water, it does not deflocculate lead arsenate as completely as may be desirable. For this reason a small quantity of a suitable colloid, such for example as the tannin or other relatively chemically inert colloids of organic origin, 125 130

hereinbefore referred to, may be added. The suspensive power of tannin and gamboge on lead arsenate in a spray solution of normal strength is indicated by the subjoined table wherein 1 gram of lead arsenate with stated amounts of tannin and gamboge were added to 250 cc. of water, and the per cent of particles of such arsenate determined in the upper 132 cc. and the lower 118 cc., respectively, of the liquid was determined after standing five minutes, viz:—

*II. Suspensive power of tannin and gamboge.*

| 15                                                                    | Top layer | Bottom layer |          |
|-----------------------------------------------------------------------|-----------|--------------|----------|
|                                                                       |           | Per cent     | Per cent |
| 1 gram lead arsenate                                                  |           | 10.25        | 89.75    |
| Ditto plus $\frac{1}{2}$ of 1% tannin                                 |           | 50.50        | 49.50    |
| Ditto plus $\frac{1}{2}$ of 1% gamboge                                |           | 26.15        | 73.85    |
| Ditto plus $\frac{1}{2}$ of 1% tannin and $\frac{1}{2}$ of 1% gamboge |           | 49.25        | 50.75    |

Neither tannin nor gamboge, or the combination of the two, appears to have any unfavorable chemical reaction on lead arsenate, as indicated by the following tests:—

*III. Amount of soluble arsenic.*

| 30 | Per cent | Lead arsenate      |                   |
|----|----------|--------------------|-------------------|
|    |          | Ditto plus gamboge | Ditto plus tannin |
|    | 0.45     | 0.45               | 0.34              |
|    | 0.45     | 0.34               | 0.34              |

Other deflocculators may be found more desirable than tannin for use with my improved spreader, but assuming tannin to be used for the purpose, the complete mixture for commercial purposes will consist of 0.32 ounces of sodium gamboge, prepared as hereinbefore described, together with 0.32 ounces of tannin, this being the proper amount for use with a spray mixture consisting of 4 lbs. of lead arsenate in 200 gallons of water. The deflocculator-spreader mixture may be added to the powdered lead arsenate at the factory or it may be sold to the consumer for addition to the spray mixture in the field. Actual field tests of a spray mixture with such deflocculator-spreader mixture added show that the surfaces of apples, for example, when sprayed in the ordinary way, are uniformly coated with the lead arsenate. It should furthermore be noted that gamboge-tannin in the amount of 0.04 lb. to 200 gallons shows no alkalinity.

The chemical composition of gamboge, so far as I am aware, is unknown. I have found, however, that it includes constituents that are respectively soluble and insoluble in water. If the raw gum of commerce be boiled with water, no alkali being used, a yellow opalescent solution of certain of the constituents of the gum is formed from which the insoluble constituents may be separated by decantation. A test of the

solution thus obtained does not indicate that such soluble constituents are particularly effective in reducing the surface tension of the watery vehicle. However, if sodium hydroxide in approximately the proportion indicated above for use with the original gum be added to such solution, very satisfactory spreading action is secured. The insoluble constituents if similarly reacted on with sodium hydroxide when used in an amount approximating from 5 to 50 per cent of the arsenate of lead powder, have a marked spreading effect. In the absence of a better general term I have used herein the name gamboge to designate inclusively the gum commercially known under this name, the constituents of such gum or such alkali metal salt thereof as will have the spreading action described above.

In conclusion I should state that while I have hereinbefore referred to the use of my improved spreader, specifically sodium gamboge, with insecticidal spray mixtures wherein lead arsenate is used as the insecticide proper, the effect of such spreader in reducing the surface tension of the liquid vehicle is not limited to this particular spray composition nor to use with spray compositions merely. On the contrary, there are many other industrial applications which need not here be enumerated for the use of such a compound.

The other gum resins hereinbefore named are prepared for use as spreaders in substantially the same manner as gamboge, to which the foregoing detail description particularly relates. I have found, however, that the alkaline derivatives of such other gum resins are equal in effect to the gamboge derivatives only when used in larger amounts. For example, two pounds of the sodium compound of olibanum in 200 gallons of water will have the same effect as two pounds of sodium gamboge (see Table I ante), but two-tenths of a pound of such first named compound will not be nearly as effective as the corresponding smaller amount of sodium gamboge.

Other forms may be employed embodying the features of my invention instead of the one here explained, change being made in the form or construction, provided the elements stated by any of the following claims or the equivalent of such stated elements be employed, whether produced by my preferred method or by others embodying steps equivalent to those stated in the following claims.

I therefor particularly point out and distinctly claim as my invention:—

1. The method of reducing the surface tension of a watery vehicle in various industrial applications, which consists in adding thereto a gum-resin derivative, substantially as described.

2. The method of reducing the surface tension of a watery vehicle in various industrial applications, which consists in adding thereto an alkali metal derivative of a gum-resin, substantially as described. 5
3. The method of reducing the surface tension of a water vehicle in various industrial applications, which consists in adding thereto a derivative of gamboge. 10
4. The method of reducing the surface tension of a watery vehicle in various industrial applications, which consists in adding thereto an alkali metal derivative of gamboge. 15
5. The method of reducing the surface tension of a watery vehicle in various industrial applications, which consists in adding sodium gamboge thereto. 20
6. The method of increasing the spreading quality of an insecticidal spray mixture of the character described, which consists in adding gamboge thereto. 25
7. The method of increasing the spreading quality of an insecticidal spray mixture of the character described, which consists in adding thereto an alkali metal salt of gamboge. 30
8. The method of increasing the spreading quality of an insecticidal spray mixture of the character described, which consists in adding sodium gamboge thereto. 35
9. A composition of matter for insecticidal use comprising an insoluble metallic arsenate and gum-resin derivative. 40
10. A composition of matter for insecticidal use comprising an insoluble metallic arsenate and gamboge. 45
11. A composition of matter for insecticidal use comprising lead arsenate and a relatively smaller amount of gamboge. 50
12. A composition of matter for insecticidal use comprising lead arsenate, a deflocculating agent, and gamboge, both of the latter in comparatively small amounts.
13. A composition of matter for insecticidal use comprising lead arsenate, tannin and gamboge, both of the latter in comparatively small amount.
14. A composition of matter for insecticidal use comprising lead arsenate, approximately one-half of one per cent. of tannin and approximately one-half of one per cent of gamboge.

Signed by me this 4th day of December, 1923.

HARRY B. GOODWIN.